

## UNITED STATES PATENT OFFICE

2,105,278

## WAVE-STILLING OIL

Johan Leonard van der Minne, Amsterdam, Netherlands, assignor to Shell Development Company, San Francisco, Calif., a corporation of Delaware

No Drawing. Application December 4, 1934, Serial No. 755,932. In the Netherlands December 5, 1933

7 Claims. (CL. 87--9)

This invention pertains to the preparation of mineral oil compositions suitable for use as wave-stilling oils.

It has been known to use for this purpose mineral, animal or vegetable oils, or their mixtures, and especially mixtures of mineral oils with fats or vegetable oils containing considerable amounts of oleic acid. The wave-stilling properties of such mixtures were ascribed to the effect of fats or of oleic acid.

It has now been found that the ability of oil mixtures to form a strong film on the surface of the water depends mainly on two factors: first, on the nature of the oil forming the base of the wave-stilling composition, and, second, on the presence in said composition of highly capillary-active organic acids, that is, acids having the property of considerably lowering the interfacial tensions when added in small amounts, especially such as the higher carboxylic acids.

With regard to the nature of the oil forming the base of the mixture, vegetable and animal oils have the drawback of not flowing easily at winter temperatures and are on this account inferior to mineral oils. However, not all mineral oils are equally suitable for the purposes of this invention, since the film formed by some of them on the surface of the water breaks more easily than that formed by other oils. It has now been found that the strongest film is formed by oils poorest in non-aromatics (those components of the oils which do not react with sulphuric acid), and it is therefore proposed, according to this invention, to use such oils in wave-stilling compositions.

Some oils, such as certain oils from the East Indies or from California, are naturally poor in non-aromatics, and their distillates and residues may often be used for wave-stilling oils without further treatment. Other oils are richer in non-aromatics, and therefore only some of their fractions may be used for that purpose. Thus, extracts obtained from refining mineral oils with selective solvents such, for example, as the Edelenau extract, the nitro-benzol extract, the cresol extract, the beta-beta-dichlor-ethyl ether and other extracts, were found to be very suitable because of their low non-aromatic content and of their cheap price. An oil of low non-aromatic content may be hereby defined as an oil at least 50% of which is soluble in three volumes of 98% sulphuric acid. It is evident, then, that mineral oils of California or East-Indian origin can especially well be used as sources of highly effective

wave-stilling oils, when their aromatic components are concentrated by solvent extraction.

According to the invention, these mineral oils of low non-aromatic content must be preferably mixed with some oil-soluble organic acid having a high interfacial tension, such, for example, as the higher carboxylic acids, like oleic, palmitic, or stearic acids, which should preferably have at least 16 carbon atoms to the molecule. Products such as rancid oil or liquid rosin, containing carboxylic acids, or any other organic acid having the property of lowering the interfacial tension, such, for example, as abietic acid, may be equally well used in wave-stilling oil compositions. The quantity in which these acids, or other non-hydrocarbon oil soluble compounds having the property of lowering the interfacial tension, or substances in which they are contained, should be added to wave-stilling compositions, depends chiefly on the characteristics of the oil forming the base of such compositions. In general, when using an oil of low non-aromatic content, as defined above, which possesses good film-forming qualities in itself, it is not necessary to add more than about 5% of, for example, a carboxylic or abietic acid to the oil. If the non-aromatic content of the oil is decreased still further, so that, for example, 60% of its components are soluble in concentrated sulphuric acid, the quantity of the substance having the property of lowering the interfacial tension added to such oil may correspondingly be decreased.

The following example of a wave-stilling oil composition may be given to illustrate this invention:

|                                 | Percent |
|---------------------------------|---------|
| Edelenau extract of kerosene    | 32      |
| Edelenau extract of spindle oil | 48      |
| Liquid rosin                    | 20      |

The modes of operation by which the present wave-stilling oil may be usefully applied are well known to those skilled in navigation.

Although heavy ground waves will not subside with the use of oil, the latter reduces the breaking of waves to a considerable degree. Oil on water, therefore, although incapable of creating a calm, is effective in producing a relatively smooth water-surface within the area of application by preventing the formation in said area of breaking waves or combers especially dangerous for navigation.

I claim as my invention:

1. A wave-stilling oil composition comprising an extract obtained from treating mineral oil

with a selective naphthenic solvent and at least 50% of which is soluble in 98% sulfuric acid, and a carboxylic acid having the property of lowering the surface tension of water.

5. 2. The composition of claim 1, in which the organic acid is a carboxylic acid having at least 16 carbon atoms to the molecule.

3. The composition of claim 1, in which the organic acid is selected from the following group:

10 10. oleic acid, palmitic acid, stearic acid.

4. The composition of claim 1, wherein the organic acid is the abietic acid.

5. A wave-stilling oil composition comprising 80% of a hydrocarbon oil soluble in liquid SO<sub>2</sub> and 20% of liquid rosin.

6. A wave-stilling oil composition comprising 80% of a mineral oil distillate soluble in liquid SO<sub>2</sub> and 20% of liquid rosin.

7. A wave-stilling oil composition consisting of about 32% of liquid SO<sub>2</sub> soluble portion of kerosene, about 48% of liquid SO<sub>2</sub> soluble portion of spindle oil, and about 20% of liquid rosin.

10

JOHAN LEONARD VAN DER MINNE.